

Aug. 8, 1950

D. MAPES ET AL

2,517,584

METHOD OF FORMING RECEPTACLES

Filed Oct. 26, 1946



Inventors

Daniel Mapes

Walter G. Sylvester

Ralph P. Hayes

By J. William Carson Attorney

## UNITED STATES PATENT OFFICE

2,517,584

## METHOD OF FORMING RECEPTACLES

Daniel Mapes, West Caldwell, Walter G. Sylvester, Jersey City, and Ralph P. Hayes, Orange, N. J., assignors to Specialties Development Corporation, Belleville, N. J., a corporation of New Jersey

Application October 26, 1946, Serial No. 705,932

3 Claims. (Cl. 29—148.2)

1

The present invention relates to methods of forming metallic receptacles, and more particularly to the provision of receptacles formed of a metal which has one heat conductive characteristic having a layer of metal at the bottom thereof which has another heat conductive characteristic.

The invention is concerned with, but not limited to, the formation of stainless steel receptacles, which have poor heat conductive characteristics, having a relatively thick layer of copper on the bottom thereof adapted to render the bottom of the receptacle highly heat conductive. The layer of copper covers the bottom of the receptacle and extends around the curved corner portions joining the bottom and side walls of the receptacle. The layer is substantially of uniform thickness at the bottom and is of gradually diminishing thickness at the corner portions.

Heretofore receptacles of the foregoing type have been made by electroplating layers of copper to the bottom of stainless steel receptacles. The methods employed in forming such layers necessitated complicated electroplating apparatus and chemical treatments which required accurate controls or highly skilled labor. Also, the quantity of current required to so electroplate the receptacles was substantially high and made the process relatively expensive.

An object of the present invention is to provide a novel, inexpensive method of making receptacles of the foregoing character.

Another object is to provide a simple method of making such receptacles which does not require complicated apparatus or controls and can be performed by unskilled labor.

Another object is to provide a method of making such receptacles wherein the dimensions of the layer on the bottom are accurately controlled in a simple manner.

A further object is to prevent distortion of the bottom of the receptacle while the layer is applied thereto.

Other and further objects of the invention will be obvious upon an understanding of the illustrative embodiment about to be described, or will be indicated in the appended claims, and various advantages not referred to herein will occur to one skilled in the art upon employment of the invention in practice.

In accordance with the invention, the foregoing objects and advantages are accomplished by forming a sheet-metal blank having a depressed central portion, establishing a pool of molten metal in the depressed central portion, solidifying the molten metal and bonding the same to the blank, and re-forming the central portion to pro-

2

vide a substantially flat bottom for a receptacle having a layer of metal at the underside thereof. In order to provide a side wall for the receptacle, the central portion is surrounded by an annular marginal portion which is re-formed after the layer of metal is bonded to the blank. This marginal portion preferably extends downwardly with respect to the depressed central portion.

In the accompanying drawing:

10 Figure 1 is a side elevational view illustrating a receptacle in the form of a cooking pot embodying the present invention.

15 Figure 2 is a side elevational view illustrating a receptacle in the form of a frying pan or skillet embodying the present invention.

16 Figure 3 is a plan view of a metallic disc adapted to be formed into a receptacle.

20 Figure 3a is a sectional view of the disc taken along the line 3a—3a on Figure 3.

25 Figure 4 is a sectional view illustrating the disc drawn into a cup-shaped blank.

Figure 5 is a sectional view illustrating the blank formed with a depressed central portion, the annular marginal portion extending downwardly with respect to the depressed portion.

25 Figure 6 is a sectional view of the blank shown in Figure 5 with a pool of molten metal established in the depressed portion and the blank supported for the bonding operation.

30 Figure 7 is a sectional view illustrating the blank after being re-formed to provide a receptacle body having a flat bottom, with the layer of metal bonded to the underside thereof and having tall side walls.

35 Figure 8 is a sectional view of a modified blank provided with a raised dome portion at the center of the depression.

40 Figure 9 is a sectional view illustrating a receptacle body having a flat bottom with the layer of metal bonded to the underside thereof and having short side walls.

45 Referring to the drawings in detail and more particularly to Figure 1, there is shown a receptacle in the form of a deep cooking pot 10 having carrying handles 11 secured thereto. The body 12 of the pot is formed of stainless steel and the bottom portion thereof has bonded thereto a layer of copper 14 which is of substantially uniform thickness at the bottom and gradually diminishes in thickness at the rounded corner joining the bottom and the side wall of the pot (Figure 7). While stainless steel is a poor conductor of heat, the high heat conductivity of the copper layer makes the bottom of the pot highly heat conductive and tends to uniformly distribute

the heat transferred through the layer of stainless steel.

In Figure 2 a stainless steel receptacle is shown in the form of a frying pan or skillet 10a having a handle 11a secured thereto and having a layer of copper 12a at the bottom portion thereof.

The receptacles shown in Figures 1 and 2 illustrate, by way of example, articles adapted to be formed by employing the methods of the present invention, it being understood that the invention is applicable to other forms of cooking vessels or utensils and to receptacles utilized for other purposes.

The method of forming the receptacle shown in Figure 1 is illustrated more particularly in Figures 3 to 7. This method comprises forming a substantially circular disc or blank 15 (Figures 3 and 3a) from a sheet of stainless steel and drawing the blank 15 into a cup 16 (Figure 4) having a bottom 17 and an annular marginal portion in the form of a side wall 19 surrounding the bottom. During the drawing operation or by a subsequent operation, the bottom 17 is formed with a circular depressed central portion 20 and an annular downwardly and inwardly inclined zone 21, as viewed in Figure 5, to provide a recess 22. Rounded corner portions 23 join the zone 21 and the side wall 19.

In order to apply a copper layer, the cup 16 is placed on a tubular cylindrical support or ring 24 which engages the rounded portions 23 at the interior of the cup as shown in Figure 6. The support is placed on a surface 25, which may be the floor of a furnace or a conveyor adapted to move the support 24 through a furnace. It will be noted that the support 24 is of a height to maintain the free edge of the side wall 19 out of contact with the surface 25.

A charge 26 comprising metallic copper in any suitable form and a suitable brazing flux is placed in the recess 22. The charge is heated by placing the support 24 with the cup 16 thereon in a furnace supplied with a reducing atmosphere and maintained at a temperature to melt the copper and thereby to establish a pool of molten copper in the recess.

The temperature in the furnace is reduced to a desired value while maintaining the reducing atmosphere. At this temperature the charge becomes solidified and the stainless steel can be quenched to retain its annealed state to facilitate further drawing thereof.

The cup is then redrawn to reduce its diameter and to elongate its side wall 19. This is accomplished by shaping the corner portions 23 and the outer peripheral portion of the zone 21 into a portion of the side wall; shaping the remainder of the zone 21 and the outer peripheral zone of the central portion 20 into rounded corner portions 31; and shaping the remainder of the central portion into a flat bottom 30 joined to the side wall 19 by the rounded portions 31, as shown in Figure 7.

The body of the receptacle 10 so shaped will have a layer of copper of substantially uniform thickness at its bottom 30, while the corner portions 31 will have a layer of copper diminishing in thickness in the direction approaching the side wall 19.

By way of example, the blank 15 may have a diameter of about sixteen inches and a thickness of about one-sixteenth of an inch. The cup 16 shaped from the blank will have a diameter of about eight inches and a height of about four and one-half inches. The depressed portion 20 may

have a diameter of about five inches and the annular zone 21 may have a width of about one inch, being inclined with respect to the portion 20 at about twenty degrees to provide a recess 22 having a depth of about one-quarter of an inch. The rounded corner portions 23 joining the side wall 19 and the zone 21 may have a radius of about one-half of an inch.

The charge 26 of copper and brazing flux placed in recess 22 may weigh about one pound and provides a pool of molten metal having a depth of about three-sixteenths of an inch. When the cup 16 is redrawn to the shape shown in Figure 7 it has a diameter of about six inches and a height of about five and one-half inches. The layer of copper 12 at the underside of the bottom 30 will have a thickness of about three-sixteenths of an inch. It will be understood that where a thicker or thinner layer of copper is desired the weight of the charge may be varied accordingly.

Referring to Figure 8, there is shown a cup 16 formed with a modified depressed central portion having a substantially shallow dome 20a. By being so shaped the recessed bottom of the cup is strengthened to prevent sagging thereof at temperatures to which the cup is subjected while in the furnace to melt the charge 26.

By increasing the height of the dome a layer of copper of a desired varying thickness may be deposited on the bottom or a layer may be deposited which is in the form of a ring to concentrate the heat transferred at the peripheral portions of the bottom.

The receptacle 10a shown in Figure 2 may be formed by practicing the methods described in connection with Figures 3 to 8 inclusive and thereafter cutting away a portion of the side wall 19 to provide a receptacle body having a side wall 36 of a desired height, as shown in Figure 9.

While the present invention has been described in connection with depositing a layer of copper on stainless steel, it will be understood that the methods described herein can be utilized for bonding a layer of other nonferrous metals to a receptacle body formed of other ferrous or nonferrous metals.

From the foregoing description, it will be seen that the present invention provides a novel, practical and economical method of applying a layer of metal to receptacle body formed of another metal. The shape of the recess is such that a charge of metal and flux can be readily melted and solidified therein to provide a smooth deposit of sound metal, which layer upon re-forming of the receptacle body remains securely bonded thereto, is of a desired thickness at the bottom and side wall of the receptacle. The contour of the cup or blank formed with the recess for receiving the charge permits controlled expansion and contraction thereof during the brazing step, thus maintaining control over the dimensions of the cup or blank and the quantity and distribution of the metal brazed thereon.

By practicing the methods described herein, improved receptacles, such as cooking utensils and the like, can be produced in a rapid and inexpensive manner. These receptacles are light in weight, rugged in construction, and can readily withstand any rough usage to which they may be subjected.

As various changes may be made in the details set forth herein, without departing from the spirit and scope of the invention and without sacrificing any of its advantages, it is to be understood that all matter herein is to be interpret-

ed as illustrative and not in any limiting sense.

It is also to be understood that the following claims are intended to cover all the generic and specific features of the invention herein described and all statements of the scope of the invention which, as a matter of language, might be said to fall therebetween.

We claim:

1. The method of forming receptacles, which comprises forming a generally circular sheet metal blank of substantially uniform thickness having an annular inwardly and downwardly extending zone and having a central depressed portion surrounded by the zone, establishing a pool of molten metal on the blank of a depth to cover the central portion and to at least partially cover the annular zone, solidifying the molten metal to cause the same to be bonded to the blank, and drawing the annular zone to form a curved annular corner and a side wall portion of smaller diameter than that of the blank, the annular zone being drawn in a direction whereby the central portion constitutes the exterior of the bottom of a receptacle and the corner portion is provided at its exterior with a layer of bonded metal diminishing in thickness from the bottom to the wall portion.

2. The method of forming receptacles, which comprises forming a cup-shaped sheet metal blank of substantially uniform thickness having a side wall and a bottom provided with an annular inwardly and downwardly extending inclined zone and a central depressed portion surrounded by the zone, establishing a pool of molten metal on the blank of a depth to cover the central portion and to at least partially cover the annular zone, solidifying the molten metal to cause the same to be bonded to the blank, and drawing the blank to reduce its diameter and to form the inclined zone into a curved annular corner and a portion of the side wall, the blank being drawn in a direction whereby the central portion constitutes the exterior of the bottom of a

receptacle and the corner portion is provided at its exterior with a layer of bonded metal diminishing in thickness from the bottom to the side wall.

3. The method of forming receptacles, which comprises forming a cup-shaped sheet metal blank of substantially uniform thickness having a side wall and a bottom provided at the exterior thereof with an annular inwardly and downwardly extending inclined zone and a central depressed portion surrounded by the zone, establishing a pool of molten metal on the blank of a depth to cover the central portion and to at least partially cover the annular zone, solidifying the molten metal to cause the same to be bonded to the blank, and drawing the blank to reduce its diameter and to form the inclined zone into a curved annular corner and a portion of the side wall, the blank being drawn in a direction to push the bottom outwardly with respect to the side wall whereby the central portion constitutes the exterior of the bottom of a receptacle and the corner portion is provided at its exterior with a layer of bonded metal diminishing in thickness from the bottom to the side wall.

DANIEL MAPES.

WALTER G. SYLVESTER.

RALPH P. HAYES.

#### REFERENCES CITED

The following references are of record in the file of this patent:

#### UNITED STATES PATENTS

| Number    | Name    | Date           |
|-----------|---------|----------------|
| 1,879,212 | Hainlen | Sept. 27, 1932 |
| 2,272,609 | Kennedy | Feb. 10, 1942  |
| 2,359,477 | Hoern   | Oct. 3, 1944   |

#### FOREIGN PATENTS

| Number  | Country | Date          |
|---------|---------|---------------|
| 338,211 | Germany | June 16, 1921 |